

## UNITED STATES PATENT OFFICE

1,958,949

MANUFACTURE OF ARTIFICIAL MATERIALS  
FROM CELLULOSE SOLUTIONS

Anton Lely, Aintree, England, assignor, by mesne assignments, to American Enka Corporation, Wilmington, Del., a corporation of Delaware

No Drawing. Application July 14, 1931, Serial No. 550,815. In Great Britain January 14, 1931

## 6 Claims. (Cl. 106—40)

This invention consists of improvements in the manufacture of artificial materials from cellulosic solutions and has particular reference to the manufacture of artificial silk from solutions of viscose.

Numerous proposals have been made for modifying the materials from which artificial silk is made, or for modifying the character, quality and appearance of the finished artificial silk by additions to the material from which the artificial silk is made.

Thus it has been proposed to modify the characteristics of artificial materials manufactured from cellulosic solutions by incorporating in the viscose or similar solution of cellulose insoluble organic liquids, or insoluble or difficultly soluble, non-volatile, difficultly volatile or readily volatile substances and these additions have been made to the spinning solutions in emulsion-like, suspension-like or colloidal form. Many of the substances mentioned above are markedly water-repellent and consequently tend to produce artificial products which lack the desirable quality of softness. In addition, a number of the substances it has been proposed to add to cellulosic solutions are unstable and tend to undergo change thus producing imperfections on the exterior of the finished materials.

It has now been found that the above-mentioned disadvantages may be avoided by selecting suitable substances for addition to viscose solutions or the like. Thus when lanoline, adeps lanæ (wool fat) is incorporated in viscose solutions an artificial silk is obtained which is remarkable for its softness and other good qualities. This result is probably attributable to the fact that lanoline while possessing fatty properties is not a true fat and is not liable to turn rancid and is not water repellent but on the contrary is capable of absorbing considerable quantities of water.

The present invention accordingly includes a process for the manufacture of artificial materials from cellulosic solutions in which the said solutions have disseminated through them prior to the spinning or extrusion operation adeps lanæ (wool fat).

The wool fat may be dissolved in a solvent therefor and then disseminated through the viscose or other cellulosic solution.

Among the solvents which may be employed are benzene, carbon tetrachloride, oil of turpentine or the like. Particularly good results are obtained from solutions of viscose or the like to which a solution of adeps lanæ (wool fat) in pine

oil has been added. It has been found that the properties of products obtained from cellulosic solutions in which pine oil solutions of lanoline have been incorporated depend on the proportion of the solution added and by varying the proportion of the solution the lustre of the product may be varied from very dull to the normally high lustre.

Quantities of wool fat amounting to 0.5% (reckoned on the cellulose) produce excellent results. For most purposes it is preferable to employ amounts of edeps lanæ (wool fat) not exceeding 3 to 4% (reckoned on the cellulose).

The solvent for the wool fat may be employed in a quantity many times that of the wool fat itself and preferably in amounts exceeding three times that of the wool fat.

This invention is applicable to the production of artificial silk by the viscose process, the acetyl cellulose process, the cuprammonia process or any other process in which a solution of cellulose or an ester or ether of cellulose is extruded into threads or filaments. The invention also includes the manufacture of horse hair, films or ribbons by the extrusion process.

The following examples illustrate methods of carrying the invention into effect:

## Example 1

Adeps lanæ (wool fat) is dissolved in four times its weight of benzene and this solution is emulsified in an approximately equal volume of viscose in an emulsifying apparatus. The mixture so prepared is gradually diluted with further quantities of viscose solution to form a uniform emulsion. The relative amounts of wool fat solution and viscose are chosen so as to yield a final solution in which the wool fat content amounts to 2% and the benzene content 8% reckoned on the cellulose content.

After the viscose solution has been allowed to ripen it is spun in the normal manner employing the usual precipitating baths.

## Example 2

One part by weight of wool fat is dissolved in nine parts by weight of oil of turpentine (pine oil brand). To 1000 kilograms of viscose containing 7.2% cellulose and 6.5% of alkali is added with emulsification 7 kilograms of the wool fat—turpentine emulsion and the whole is allowed to stand until ripe for spinning. The subsequent processes are carried out in known manner.

I claim:

1. In a process for the manufacture of de-lustered artificial silk filaments from viscose solu-

tions, the step which includes emulsifying in the viscose solution, adeps lanæ (wool fat) which has previously been dissolved in a solvent of the class consisting of pine oil, benzene and carbon tetrachloride.

2. In a process for the manufacture of de-lustered artificial silk filaments from viscose solutions, the step which includes emulsifying in the viscose solution, adeps lanæ (wool fat) which has previously been dissolved in pine oil.

3. In a process for the manufacture of de-lustered artificial silk filaments from viscose solutions, the step which includes emulsifying in the viscose solution, adeps lanæ (wool fat) which has previously been dissolved in benzene.

4. In a process for the manufacture of de-lustered artificial silk filaments from viscose solutions, the step which includes emulsifying in the viscose solution, adeps lanæ (wool fat) which has previously been dissolved in carbon tetrachloride.

5. In a process for the manufacture of de-lustered artificial silk filaments from viscose solutions, the step which includes emulsifying in the viscose solution, adeps lanæ (wool fat) which has previously been dissolved in a solvent of the class consisting of pine oil, benzene and carbon tetrachloride, the amount of adeps lanæ being in the range of .5% to 4% reckoned on the cellulose content.

6. In a process for the manufacture of de-lustered artificial silk filaments from viscose solutions, the step which includes emulsifying in the viscose solution, adeps lanæ (wool fat) which has previously been dissolved in a solvent of the class consisting of pine oil, benzene and carbon tetrachloride, the amount of adeps lanæ being at all times less than one third of the amount of the said solvent.

ANTON LELY.

80

85

90

95

100

105

110

115

120

125

130

135

140

145

150

25

30

35

40

45

50

55

60

65

70

75